

Patented Feb. 20, 1934

1,948,308

## UNITED STATES PATENT OFFICE

1,948,308

## METHOD OF MAKING MAGNETIC BODIES

Charles C. Neighbors, Chicago, Ill., assignor to  
Western Electric Company, Incorporated, New  
York, N. Y., a corporation of New York

No Drawing. Application December 11, 1931  
Serial No. 580,503

11 Claims. (Cl. 175—21)

This invention relates to a method of making magnetic bodies and more particularly magnetic bodies made of finely divided magnetic material.

An object of the invention is to provide a method of producing magnetic bodies having improved magnetic properties and low energy losses.

Magnetic cores formed of finely divided and individually insulated particles of magnetic material are extensively used in loading coils for im-

10 proving the transmission characteristics of telephone lines. In the construction of such cores the finely divided magnetic material is mixed with an insulating material which serves also as a binder and the mixture is subjected to a

15 pressure of substantially 200,000 pounds per square inch to form the component material into a substantially homogeneous mass having a high degree of mechanical strength. In cores of this type, particularly those in which the magnetic

20 material is a nickel-iron alloy, the insulating material must be of such a character as to be able to withstand the heat-treatment and mechanical operations to which the material is subjected in forming the cores and developing the mag-

25 netic properties of the material.

In accordance with one embodiment of the present invention, magnetic material in finely divided form is mixed with a portion of insulating material consisting of a water soluble organic acid, such as tartaric acid, and additional in-

30 gredients, such as sodium silicate, talc and kaolin. The insulating material is thoroughly mixed with the particles of magnetic material and the entire mass is evaporated to complete dryness. The

35 coated particles are then mixed with a second portion of the insulating material and again the mass is evaporated to complete dryness. A third coating is then applied in the same manner and the material is then pressed into suitable cores which

40 are annealed to relieve the mechanical strains in the material and improve the magnetic properties of the cores.

In practicing the present invention, the magnetic material is preferably prepared from a brittle alloy containing nickel and iron, with or without the addition of other constituents, and commonly known as "permalloy". The alloy may be prepared in the manner described in Patent No.

45 1,669,649 issued May 15, 1928 to C. P. Beath and H. M. E. Heinicke, wherein approximately 81 parts of nickel and 19 parts of iron are melted together in an oxidizing atmosphere, the resulting alloy being poured into a mold. The alloy thus prepared is rolled while hot into relatively thin

50 slabs which are quenched rapidly to produce a

fine crystalline structure which is desirable since the disintegration of the material takes place at the crystal boundaries and, consequently, the smaller the size of the crystals the finer the dust which can be produced therefrom. The slabs 60 are then reduced to a finely divided form in any suitable manner and the finely divided alloy is subsequently reduced to a dust by pulverizing it in an attrition or ball mill.

The dust from the attrition or ball mill is then 65 sifted and the portion passing through a 120-mesh screen is placed in a closed container and annealed at a temperature of approximately 885° C. The annealed dust is removed from the container in the form of a cake, which is again reduced to a powder by crushing it in a rotary crusher and subsequently grinding it in an attrition mill, the ground dust is again sifted through a 120 mesh screen and the dust passing the screen is then mixed with the insulating com- 70 position as described hereinafter. It should be understood, however, that the present invention is independent of the particular magnetic metal or alloy employed, and of the manner of preparing the metal or alloy. The term "magnetic 75 metal", as used herein, is therefore intended to include any magnetic metal or alloy of metals suitable for use in connection with the present invention, regardless of its composition or method of preparation.

As an example of an insulating composition suitable for the purposes of the present invention, the following formula is given:

|                 | Pounds |
|-----------------|--------|
| Tartaric acid   | .30 90 |
| Sodium silicate | 1.05   |
| Powdered talc   | .75    |
| Kaolin          | .75    |
| Water           | 12.00  |

The ratio of acid to sodium silicate, as given in the above formula, is 1:3½ but may range from 1:3 to 1:8 or upwards, the effectiveness of the insulation decreasing somewhat as the ratio of acid to sodium silicate decreases from that given in the above formula. The ratio of the solid materials (talc and kaolin) to the water-soluble materials (acid and sodium silicate) may be varied widely, as may also the ratio of water to the other ingredients, the water being used merely to dissolve the water-soluble materials and to give the desired consistency to the mixture of insulating composition and dust.

The kaolin specified in the above formula is a binder and has the function of preventing cracks in the finished core parts, in addition to

*may be omitted*

being a rather effective insulating material. In certain cases it may be omitted, depending upon the characteristics desired in the finished core parts.

5 The permalloy dust thus obtained is thoroughly mixed with a portion of insulating material. It has been found that best results are obtained by applying the insulating material in two to five successive steps. This makes it possible to use a smaller amount of insulating material and still obtain a better insulation of the particles. The smaller amount of insulating material used also increases the permeability of the magnetic body because permeability is proportional to the amount of insulating material used. The total amount of insulating material may be as low as  $\frac{1}{2}\%$  of the amount of dust used according to the permeability desired.

For convenience the total amount of insulating material used is usually divided into a number of parts equal to the number of coatings to be applied, although it has been found by experiment that when the coatings are applied in successively increasing amounts better results are obtained than when the coatings are applied in equal amounts. As an example of using successively increasing amounts of insulating material per coating when the amount of insulating material is 3.2% of permalloy dust by weight, a quantity of permalloy dust is first mixed with a quantity of insulating material comprising .50% of the quantity of dust by weight. The mixture is then evaporated to a condition of complete dryness in order to obtain the maximum insulating resistance and is stirred constantly to prevent caking and to insure a thorough coating of the individual dust particles. To obtain a complete drying of the magnetic material, its temperature may be raised to  $120^{\circ}\text{C}.$ , and even much higher temperatures may be used without injury to the material. The material after being thoroughly dried has a very low affinity for water, so that no special protection need be provided against the absorption of water by the material.

After the application of the first coating, the coated particles are again mixed with about 1.0% of the insulating material in the same manner and the material is then again evaporated to dryness. In applying the third coat, 1.7% of insulating material is added to the double coated particles and the mixture is again evaporated to complete dryness.

It is important in this method that each coating be rendered insoluble by drying before the next coating is applied, otherwise the application of a subsequent coating would tend to redissolve the previously applied coating and destroy the effectiveness of the multiple coating.

60 The insulated dust is sifted through a 16-mesh screen, placed in a mold and compressed into core parts under a pressure of approximately 200,000 pounds per square inch. The core parts are then transferred to an annealing furnace where they are annealed to relieve the internal stresses set up by the pressing operation and thereby to produce a core having low hysteresis loss and high permeability. The annealing temperature used is preferably about  $500^{\circ}\text{C}.$ , but a temperature as high as  $565^{\circ}\text{C}.$  may be used without destroying the effectiveness of the insulation. Where a temperature of  $500^{\circ}\text{C}.$  is used, the core parts are preferably raised to that temperature in about twenty minutes and maintained at such temperature for about five minutes. These

annealing temperatures and periods may vary with cores of different sizes. If higher annealing temperatures are used, the time should, of course, be proportionately shortened and vice versa.

The drying and annealing temperatures apparently drive off substantially all of the volatile constituents of the material, including the organic acid, in the form of gases, with the result that the annealed core parts contain only the end-products of the heating process and contain no water-absorbent substances. This makes it unnecessary to wash and dry the core parts after annealing to remove such water-absorbent substances. The tartaric acid used is a very weak oxidizing agent and, since it volatilizes at a relatively low temperature, very little oxidation of the metal takes place during the annealing operation. Such oxidation may be objectionable in some cases since it appears to affect unfavorably the magnetic qualities of the finished cores.

As an example of the effect of the triple coating of the dust particles, the following results of tests made on core rings commonly referred to as 75 permeability cores are given. Three batches of core rings were made up and a single coating of insulating material was applied to one set, a double coating was applied to the second set, and a triple coating was applied to the third set, with the following results:

| Number of coatings | Resistance in ohms | Percent of insulating material by weight of dust |
|--------------------|--------------------|--------------------------------------------------|
| 1 coating.....     | 35.0               | 2.5                                              |
| 2 coatings.....    | 390.0              | 2.4                                              |
| 3 coatings.....    | 1500.0             | 2.3                                              |

It will be noted that the total amount of insulating material used in the double coated batch of rings was less than for the single coated batch, and the total amount of insulating material used in the triple coated batch was less than used in either the single or double coated batch. Due to the high resistance of the core material when the triple coating of insulation is applied, it is evident that the energy losses due to eddy currents in the core will be extremely low.

Another test of multiple coatings was made on magnetic dust particles made in accordance with the disclosure of the patent to White et al., No. 1,787,606, January 6, 1931, using 2% molybdenum and 4% copper in the magnetic alloy from which the dust was made with the following results:

| Number of coatings | Resistance | Permeability | Eddy current constant |
|--------------------|------------|--------------|-----------------------|
| 1 coating.....     | .8         | 107.0        | 3.50                  |
| 4 coatings.....    | 8.0        | 114.5        | 1.78                  |
| 5 coatings.....    | 12.0       | 110.8        | 1.22                  |

The total amount of insulation in each case was 1.2% of the dust by weight. These cores were considerably smaller than those of the previous example which accounts for the lower resistance of these cores. However, it will be noted that the resistance increased enormously and consistently with the increased number of coatings.

The standard amount of insulation used heretofore has been about 3.2% of the dust by weight. The use of the multiple coating indicates that

much smaller amounts of insulating materials may be used for a particular resistance of the cores and as pointed out above the less insulating material used the higher will be the permeability of the cores.

One or more core parts thus formed are then used to constitute a core to which the usual toroidal winding is applied to form a loading coil, the number of core parts used depending upon the electrical characteristics of the circuit with which the loading coil is to be associated.

In place of the tartaric acid specified in the above formula, any other suitable water-soluble organic acid may be used, although it is preferred to use a non-corrosive, non-irritating, non-oxidizing organic acid and one which leaves a non-hygroscopic residue, such as tartaric, lactic and citric acids. Other suitable acids which may be used are succinic, oxalic, and malonic acids.

The invention is not limited to the embodiments above described but may be varied widely within the scope of the following claims.

What is claimed is:

1. A method of producing a magnetic body which consists of mixing finely divided dust particles with an insulating material including an organic acid, drying the mixture, mixing a second quantity of said insulating material with the resulting product and again drying the mixture.

2. A method of producing a magnetic body from finely divided magnetic particles which consists of mixing an aqueous insulating material with said particles, forming a water insoluble dry film on the particles, mixing a second portion of said aqueous insulating material with the coated particles, and forming a second water insoluble dry film over said first film.

3. A method of producing a magnetic body from magnetic particles which consists of consecutively applying a plurality of water insoluble insulating coatings to the particles and treating the particles between the applications of the coatings.

4. A method of producing a magnetic body from magnetic particles which consists of consecutively applying a plurality of coatings of water laden insulating material to the particles and rendering each coating water insoluble before the application of the following coating.

5. A method of producing magnetic bodies from magnetic particles which consists of consecutively applying a plurality of coatings of a compound containing tartaric acid, sodium silicate, water, and an insulating material to the particles, and evaporating the water to form a water insoluble film on the particle after each coating is applied.

60

6. A method of producing a magnetic body which consists of compounding an insulating material of kaolin, sodium silicate, talc, water, and tartaric acid, mixing a quantity of the insulating material with particles of magnetic material, evaporating the material to dryness, applying a second coating of the insulating material to the coated particles and again evaporating the material to dryness.

80

7. A process of producing a magnetic body from particles of magnetic material and a given amount of insulating material including soluble ingredients, insoluble ingredients, and tartaric acid, which consists of mixing the magnetic particles with a portion of said insulating material, evaporating the mixture to dryness, repeating this process until all of the insulating material has been used, and forming the particles into a core.

85

8. A method of producing a magnetic body from particles of magnetic material which consists of compounding an insulating composition of an organic acid, sodium silicate and insoluble insulating material, mixing a quantity of the particles with the insulating composition, evaporating the mixture to dryness, mixing the resulting product with a second quantity of the insulating composition and again evaporating the mixture to dryness and forming the resulting product into a core.

95

9. A method of producing a magnetic body which consists of forming a solution of water, sodium silicate and an organic acid, suspending insoluble insulating material in the solution, mixing the resulting product with particles of magnetic material, evaporating the mixture to dryness to form an insoluble film on the particles, mixing the coated particles with a second quantity of the insulating material, and again evaporating the mixture to dryness, and subsequently forming the material into cores.

105

10. A method of producing a magnetic body from a given amount of magnetic dust and a given amount of insulating material which consists of applying the insulating material in a plurality of steps and applying a substantially greater amount of insulating material in a subsequent step than applied in a preceding step.

115

11. A method of producing a magnetic body from finely divided dust particles which consists of compounding an insulating material of solid material, sodium silicate, an organic acid and water, applying a given amount of the insulating material in successive steps and evaporating the coated particles to dryness after each application of insulating material.

125

130

CHARLES C. NEIGHBORS.

135

140

145

150

65

70

75